

F. SEARLE,

# COMPOSITE STOCK FOR MACHINE KNIVES AND METHOD OF MAKING THE SAME

APPLICATION FILED MAY 7, 1908.

925,661.

Patented June 22, 1909.



### FIG. 1.



FIG. 2.



FIG. 3.



FIG. 4.



FIGURE 57



FIG. 6

*Witnesses.*

Frank C. Woodland

Ella P. Blenner

### *Inventor.*

Frederick Sears  
By Chas. H. Burleigh  
Attorney

# UNITED STATES PATENT OFFICE.

FREDERICK SEARLE, OF WORCESTER, MASSACHUSETTS, ASSIGNOR TO COES WRENCH COMPANY, OF WORCESTER, MASSACHUSETTS, A CORPORATION OF MASSACHUSETTS.

## COMPOSITE STOCK FOR MACHINE-KNIVES AND METHOD OF MAKING THE SAME.

No. 925,661.

Specification of Letters Patent.

Patented June 22, 1909.

Application filed May 7, 1908. Serial No. 431,331.

*To all whom it may concern:*

Be it known that I, FREDERICK SEARLE, a citizen of the United States, residing at Worcester, in the county of Worcester and 5 State of Massachusetts, have invented a new and useful Composite Stock for Machine-Knives and Method of Making the Same, of which the following is a specification, reference being made therein to the accompanying drawings.

The object of my present invention is the production of a securely welded composite stock for machine knives of the double edged channel-bar pattern, more especially for the 15 ledger knives for lawn mowers, or similar knives having two turned up edges. Also, to provide a conveniently workable process whereby a double edged channel-bar knife-stock can be successfully and economically 20 manufactured, and the steel edging material efficiently affixed to the body or backing by a V-welded integration; and to practically produce a composite stock of such character that the dual cutting-edges of knives made 25 therefrom can be properly hardened and tempered without destroying the capacity of the product for being straightened or fitted after the knife is formed, or while being formed therefrom; thereby affording more perfect 30 and stronger knives of the pattern specified than heretofore produced. These objects I attain by the means hereinafter explained, and illustrated in the drawings, wherein—

Figure 1 represents a cross section of the 35 iron and steel members as primarily assembled in the fagot. Fig. 2 represents a cross section of the billet after going through the first reduction pass. Figs. 3 and 4 represent successive cross section shapes of the 40 composite bar after going through the second and third reduction passes respectively. Fig. 5 represents a cross section of the completed stock as it is issued from the final pass of the reduction rolls; and Fig. 6 is a front 45 view of a pair of reducing rolls having passes formed for producing composite knife-stock in accordance with my invention.

In a machine knife of the channel-bar shape it is desirable that the upturned lips, 50 whereon the cutting edges are formed, should be hardened and tempered, while the bar as a whole should be strong and rigid, but at the

same time sufficiently tough and bendable to permit of the knife made therefrom being 55 straightened or fitted, to eliminate the warpings and distortions incident to the hardening operations, or to properly adjust the alignment of the opposite edges. It is also essential that the lips or upturned edges be of 60 such quality and texture that they can be ground away, by successive sharpenings, quite or nearly to the bottom plate or backing. A stock made entirely of steel would of course give good cutting edges, but an all- 65 steel stock, when hardened to the required degree, cannot be successfully straightened and adjusted by bending; and furthermore an all-steel stock is comparatively expensive and may not be produced with the requisite 70 economy.

To produce composite stock of the shape specified and having the requisite qualities, and that can be manufactured with practical economy and success, my improved process 75 is as follows: I prepare a fagot (Fig. 1) of the desired length, composed of a rectangular sectioned bar I of refined wrought iron, or soft steel (of ten per cent. carbon or less) of a dimension say three-fourths inch by one and 80 three-fourths inches, more or less, and two rectangular sectioned bars S of crucible cast-steel or tool-steel, of a dimension say one inch by five sixteenths inch, more or less, which latter are placed flatwise against the 85 opposite edges 12 of the body-bar I, with their respective edges 13 projecting in either direction beyond the flat faces of said body-bar, as illustrated in Fig. 1; in which form the members, previously heated and fluxed, 90 are hammer-welded to primarily unite their adjacent surfaces sufficiently to keep the members together in place. This fagot, when properly heated, is run through a pair of reducing rolls A, B, in a pass 1 having an 95 approximately straight top and bottom, and rounded or inclined ends that compress the exterior angles of the billet and firmly weld the steel members to the opposite edges of the body-bar, reduced as at I<sup>1</sup>, with a somewhat crescentic shaped cross-section, as at S<sup>1</sup>, forming an overthrust of the upper and lower edges of the steel at the weld joint 5, as indicated in Fig. 2. The composite billet is then further reduced in a pass 2, the form of 100 105

which presents a flat at one side and a double channeled contour at the opposite side; whereby the billet is given the shape approximately as shown in Fig. 3, the intermedial portion  $I^2$  being reduced to about one half the thickness of the side portions  $S^2$ , which latter are crowded inward at the corners 6. The bar is next inverted and put through a reducing pass 3 that flattens the body or backing portion nearly to its final thickness, as at  $I^3$ , and transforms the edge portions into embryo upturned lips, as at  $S^3$ , forcing the lines of the welding into oppositely directed bird-mouth or **V**-shaped contour, as at 7, but leaving a proportional excess of thickness at the shoulder 8; the stock then having the shape approximately as indicated in Fig. 4. The bar when thus shaped is put through a final pass 4 of the rolls, whereby it is slightly reduced in its full width, the body portion flattened or further reduced to finished dimension for the backing, as at  $I^4$ , and the excess at the shoulders 8 reduced in thickness and forced upward making the upturned lips  $S^4$ , at each edge, complete and of approximately uniform thickness therewith; and disposing the **V**-shaped welding along the angle or base of the lips in such manner that the upstanding lips are substantially all hard steel, while the backing or body web is of iron or non-hardening material, as shown in Fig. 5. Thus producing a firmly united composite stock of channel-bar section, with edges that can be hardened and tempered, and with a body that will permit of the straightening, twisting, or readjustment of the alignment of the knife after it has been tempered, and with the **V**-welds of the steel-edge overlapping onto the softer material approximately along the angles, as at 9, in a manner that will avoid liability of rupture in the weld in the process of manufacture; the stock presenting hard and efficient upstanding lips along both edges.

45 The class of machine knives for which this improved composite stock is produced, and for which it is peculiarly adapted, are the ledger-knives for lawn mowers and similar mechanisms, wherein a spirally bladed revolver is arranged to shear against a straight ledger knife. The finished knife made from this cutter-stock is of approximately the same cross-section as that of the complete stock, as shown in Fig. 5; the knife being a piece of the stock of the required length, suitably hardened and tempered, and having the top edges and outer faces of the upstanding lips simply ground, on the lines  $f$  and  $t$ , for giving the desired cutting edges, and which can be re-ground and used until the entire upstanding lips are worn away, without exhausting the quality of the stock.

I am aware that a channel-bar shaped cutter stock of a non-composite nature has here-

tofore been employed, and I do not, therefore, herein broadly claim that shape, *per se*, as applied to cutters; but so far as I am aware a composite soft-bodied, dual steel-edged knife-stock of the shape and inherent structure herein described, has never been heretofore successful produced, nor a method disclosed for the practical manufacturing of such formed composite knife-stock, prior to my invention hereinbefore set forth.

What I claim and desire to secure by Letters Patent, is—

1. The method of making double-lipped composite knife-stock, which consists in applying to each of the two edges of a rectangular bar of wrought iron a bar of cast or tool steel of greater width than the thickness of the iron, condensing this composite fagot to weld and form the steel in approximately crescent shape upon the respective edges of the body-bar, reducing said bar with an excess of reduction centrally along one side; further reducing the same in channel-bar shape to form embryo lips of the steel having an excess of thickness at the shoulders where the welds embrace the edges of the iron, then rolling said reduced bar into its final double-lipped shape with the mass of steel chiefly disposed in the lips, and the welding line along the base of the lip, substantially as set forth.

2. The improvement in the method of making composite stock for dual-edged machine knives of the character specified, which consists in combining in a fagot, a rectangular sectional body-bar of iron or soft steel and two bars of crucible cast or tool steel respectively arranged with projecting edges upon the opposite edges of said body-bar, primarily uniting the same by hammer-welding, and at an initial rolling compressing the exterior projecting edges of the billet inward so as to overthrust the steel edgings in opposite crescentic form upon the body portion, then reducing the body thickness, and by successive stages subsequently forcing the steel edgings into the form of upstanding lips at the respective edges, and closing the welding lines into inwardly over-lapping bird-mouth or **V**-shaped integrations along the opposite edges of the backing body, substantially as set forth.

3. A composite stock for machine-knives of channel-bar cross-section, said stock comprising an approximately flat body-portion consisting of soft non-hardenable steel or wrought-iron, and offset upstanding longitudinal lips consisting of hardenable steel or tool-steel along each edge of said body, the body and lip portions being integrally united by oppositely disposed **V**-shaped weldings, longitudinally along the junction line of the lip and body, as set forth.

4. The within described double-edged

composite stock for machine-knives, said stock comprising a flat non-hardenable central body-strip, in combination with an up-standing outwardly inclined lip of hardenable steel uniformly applied thereto along each of the edges, said lips being of approximately the same thickness as the body-strip, and integrally united longitudinally therewith by oppositely disposed weldings located at the angle or up-turn-offset of the respective lips, substantially as set forth.

Witness my hand this fourth day of May 1908.

5

FREDERICK SEARLE.

Witnesses:

CHAS. H. BURLEIGH,  
ELLA P. BLENUS.